

## UNITED STATES PATENT OFFICE

1,977,182

CORROSION-RESISTING FERROUS ALLOY  
ADAPTED FOR FORGING AND CASTING  
PURPOSESMaurice Palmyre Fould, Paris, France, assignor  
to Societe Anonyme Des Hauts-Fourneaux,  
Forges & Acieries De Pompey, Paris, FranceNo Drawing. Application September 15, 1933,  
Serial No. 689,563. In France September 26,  
1932

3 Claims. (Cl. 75—1)

The invention relates to corrosion-resisting ferrous alloys, and more particularly to those corrosion-resisting alloys which are related to pure iron in contradistinction with the non-rusting 5 steels which contain a large proportion of special components.

The ferrous alloys of the class herein referred to are very pure ferrous alloys, which may contain 10 small amounts of copper, tungsten or molybdenum, chromium, nickel etc. They may optionally contain silicon, according as the metal is "quiet" or "foamy", but are always practically free from carbon, phosphorus and sulphur, and it is difficult, or even impossible, to cast them.

15 The present invention has for its object a ferrous alloy which resists corrosion, and can be forged or moulded, and which contains, in addition to the iron, approximately the following proportions of the following components:

20 Carbon less than 0.050%  
Manganese from 0.200 to 0.600%  
Silicon from 0.200 to 0.600%  
Phosphorus less than 0.020%  
25 Sulphur less than 0.015%  
Copper from 0.300 to 0.600%  
Tungsten from 0.010 to 0.150%

The resistance to corrosion of this metal when "quiet" is not altered by the presence of manganese, even in a large proportion, such as 30 0.600%.

35 Into the known ferrous alloys above referred to from 0.01 to 0.4% of chromium was sometimes added in order to improve the mechanical features. Inasmuch as, in the alloy according to the invention, the proportion of manganese is between 0.2 and 0.6%, it is no longer necessary to employ chromium in order to obtain the same tensile strength.

40 The alloy according to the invention, in the annealed state, shows the following mechanical features, as tested upon standard samples:

Coefficient of elasticity E from 28 to 32 kgs. 45 p. sq. mm.  
Tensile strength R from 40 to 46 kgs. p. sq. mm.  
Elongation A from 26 to 30%  
Resilience  $\rho$  more than 25 kgs.

50 The resistance of this ferrous alloy to corrosion is shown by the following test. A disc having 55.74 mm. diameter is cut in a casting and is pierced at its centre with a circular hole of 10 mm. diameter; the test piece is lathe-turned so as to provide a symmetrical bevelled outline, having a 55 constant thickness of 3 mm. within a circle hav-

ing a diameter of 20 mm., and then regularly decreasing to 1 millimetre at the periphery. The sample is then polished, cleaned, and pickled successively in concentrated baths of nitric acid and hydrochloric acid, until the crystalline texture appears, and it is finally immersed for five minutes in a solution of sulphuric acid at 30% by weight, at a temperature of 50° C. The sample is then removed and washed, and is immersed before any commencement of oxidation, in a solution of sulphuric acid at 30% by weight of acid  $\text{SO}_4\text{H}_2$  at a temperature of 17° C., in an inclined position with reference to the vessel containing the solution, and it is allowed to remain therein for 48 consecutive hours.

60 At the end of this time, the test piece is removed, and the amount of iron dissolved is determined by oxidizing the ferrous sulphate by means of potassium permanganate. The degree of corrosion is found to be comprised between 0.05 and 1 milligramme of dissolved iron per square centimeter of surface of the test piece and per 24 hours.

65 The homogeneity of this steel can be shown by a macrographic examination of a section of the rolled metal, perpendicular to the direction of rolling, that is perpendicular to the axis of the original ingot. The macrographic sample may be prepared by a prolonged attack by hot sulphuric acid or the test may be made with Baumann paper.

70 Whilst the known alloys of the above-mentioned class, whether quiet or foamy, show a great heterogeneity of structure between the centre and the periphery, the alloy according to the present invention is remarkably homogeneous.

75 Owing to the manganese, the forging quality of this alloy is improved, throughout the whole range of temperatures, as compared with the similar metals now in use.

80 Due to its composition, this alloy can be used for casting purposes, whilst the known similar alloys cannot be cast or yield blistered castings.

85 The alloy according to the invention may be produced by any of the usual metallurgical processes, and particularly in the Siemens-Martin furnace or the electric furnace, after a complete refining under a very calcareous slag, until a bath of very soft iron is obtained; the slag is then removed and a fresh calcareous slag is formed, and 90 at this time, the manganese can be introduced in any desired form, whether as silico-manganese, ferro-manganese or super-refined manganese.

95 The tungsten may be added at the same time as the manganese, or subsequently; the copper 100

105

110

may be added at any time, but it is preferably incorporated with the initial charge.

Although the said alloy is particularly useful where special resistance to sulphuric acid is required, it also shows a considerable resistance to further acid corrosive agents such as hydrochloric acid, vapours of pickling rooms, acid residual waters, etc. It also shows a greater resistance to sea water and to sea spray than iron of very great purity.

Having now described my invention what I claim as new and desire to secure by Letters Patent is:

1. A corrosion resisting iron alloy particularly adapted to resist the action of acid media, such as sulphuric acid, comprising the following constituents, in the following approximate proportions by weight:

20 Carbon..... less than 0.050%  
Manganese..... from 0.200 to 0.600%  
Silicon..... from 0.200 to 0.600%  
Phosphorus..... less than 0.020%  
Sulphur..... less than 0.015%  
Copper..... from 0.300 to 0.600%  
25 Tungsten..... from 0.010 to 0.150%  
Iron..... the rest

2. An acid resisting casting consisting of a fer-

rous alloy comprising the following constituents, in the following approximate proportions by weight:

Carbon..... less than 0.050% 80  
Manganese..... from 0.200 to 0.600%  
Silicon..... from 0.200 to 0.600%  
Phosphorus..... less than 0.020%  
Sulphur..... less than 0.015%  
Copper..... from 0.300 to 0.600%  
Tungsten..... from 0.010 to 0.150%  
Iron..... the rest 85

3. An acid resisting forged ferrous alloy comprising the following constituents, in the following approximate proportions by weight: 90

Carbon..... less than 0.050%  
Manganese..... from 0.200 to 0.600%  
Silicon..... from 0.200 to 0.600%  
Phosphorus..... less than 0.020%  
Sulphur..... less than 0.015% 95  
Copper..... from 0.300 to 0.600%  
Tungsten..... from 0.010 to 0.150%  
Iron..... the rest

MAURICE PALMYRE FOULD. 100

30 ..... 105

35 ..... 110

40 ..... 115

45 ..... 120

50 ..... 125

55 ..... 130

60 ..... 135

65 ..... 140

70 ..... 145

75 ..... 150